

Dec. 15, 1953

J. WEGMANN ET AL

2,662,807

PROCESS FOR DYEING CELLULOSE FIBERS WITH  
DIRECT-DYEING CUPRIFEROUS AZO-DYE STUFFS  
AND DYE BATHS USED THEREFOR  
Filed Nov. 7, 1951



INVENTORS

Jacques Wegmann and Karl Menzi

BY

Wendroth, Lind &

Ponack

ATTORNEYS

Patented Dec. 15, 1953

2,662,807

# UNITED STATES PATENT OFFICE

2,662,807

## PROCESS FOR DYEING CELLULOSE FIBERS WITH DIRECT-DYEING CUPRIFEROUS AZO-DYESUFFS AND DYEBAHS USED THEREFOR

Jacques Wegmann and Karl Menzi, Basel, Switzerland, assignors to Ciba Limited, Basel, Switzerland, a Swiss firm

Application November 7, 1951, Serial No. 255,247

Claims priority, application France  
November 10, 1950

17 Claims. (Cl. 8—42)

1

This invention is based on the observation that cellulose fibers can be dyed in a very advantageous manner with direct dyeing cupriferous or nickeliferous azo-dyesuffs, if a dyebath is used which contains an aliphatic amine having at least two nitrogen atoms each bound to two carbon atoms and at least two hydroxyl groups.

As cellulose fibers there come into consideration for example, cotton or linen, and also fibers of regenerated cellulose such as artificial silk or staple fibers, and furthermore mixtures of fibers containing cellulose fibers.

As direct dyeing cupriferous or nickeliferous azo dyesuffs there are to be understood complex copper or nickel compounds of azo-dyesuffs which possess an adequate affinity for cellulose fibers and sufficient solubility, and which can therefore be applied in dyeing by the known direct dyeing processes.

Among the aliphatic amines defined above there may be mentioned, for example, those of the general formula



in which  $\text{R}_1$  indicates a hydrogen atom, an alkyl group with at the most three carbon atoms or a hydroxymethyl group,  $\text{R}_2$  a hydrogen atom or a methyl group and  $n$  a whole number which is at the most 4 but preferably 2.

As examples may be mentioned the bases of the following composition:



M. P. 93 to 94° C.



M. P. 136 to 139° C.



M. P. 177 to 181° C.

Especially suitable among compounds of this kind is the already mentioned 1:2-di-( $\beta$ -hydroxyethylamino)-ethane of the formula



Apart from the content of an amine of the above kind, the dyebaths used in the present process may contain the usual additions which are known for dyeing cellulose materials with direct dye-

2

stuffs. They may contain, for example, besides the dyesuff, sodium sulfate and/or sodium carbonate. The liquor ratio, that is to say the ratio of the quantity of the material to be dyed to the quantity of the dye liquor is in the present process variable within especially wide limits.

The addition of the amines of the above kind to the dyebaths influences the dyeing process and the results in an unexpected manner. The amine has a strong restraining action such that only a part of the dyesuff is taken up by the fiber and the remainder, which but for the addition of amine would have been taken up, remains in solution in the dyebath. This state of equilibrium is generally reached very rapidly at any given temperature with the result that further quantities of dyesuff cannot be taken up by prolonging the period of dyeing. The extent of the restraining action of the amine is different with different dyesuff; in other respects it is dependent on the concentration, that is to say, on the content of amine in the dyebath. Even at very high dilutions, for example, with 0.1 gram of amine per liter of dyebath, a very strong action is obtained in some cases. At a concentration of 3 grams of amine per liter the maximum possible restraining action is usually obtained.

At any given amine concentration, quantity of dyesuff and quantity of material to be dyed the restraining action is constant within wide limits, that is to say, it is independent of the liquor ratio (it will be apparent from the foregoing that the amine concentration means the number of parts of amine present in 1000 parts by volume of dye liquor; that the quantity of dyesuff and the quantity of the material to be dyed mean the number of parts of these components; and that the liquor ratio means the ratio of the number of parts of the material to be dyed to the number of parts by volume of the dye liquor). Accordingly there are produced with dyebaths which are concentrated or dilute with respect to the dyesuff content therein, and which contain the same quantity of dyesuff and the same concentration of amine and, if salts such as sodium sulfate are present, the same concentration of salt, dyeings of practically the same strength on the same quantity of dyed goods.

By the addition of aldehydes, especially formaldehyde, the restraining action of the amine can be reduced, should this be desired.

The present invention constitutes a valuable advance in the art. Inter alia, it enables dyeing with direct dyeing cupriferous dyesuffs to be carried out in a specially advantageous manner.

When, for example, it is desired to dye a large quantity of textile material of the same tint and several dyeing operations are necessary for

this purpose, this can be achieved by the present process in an especially simple and controllable manner. For this purpose the dyebath is made up by incorporating therein, on the one hand, a quantity of dyestuff many times, for example, 10 times, the quantity necessary for producing the desired tint and, on the other, such a quantity of amine that only that proportion of the dyestuff present, for example, 1/16 thereof, which yields the desired strength of dyeing is taken up by the fiber. With respect to most dyestuffs the restraining action of the amine is so great that the dyestuff consumed in the first dyeing operation need not be replaced immediately or replaced with great accuracy. In general, when the dyestuff consumed in the first operation is not replaced, the second and in many cases further dyeings are so little weaker than the first dyeing that the differences in strength are not perceptible even to the eye of an expert. Accordingly, in some cases there are produced from the same dyebath without the addition of further dyestuff in two or more operations practically identical tints. It will also be apparent that even in cases where (after one or more dyeing operations) it is necessary to add fresh dyestuff for the subsequent dyeing operations, the quantity of the dyestuff to be added can be chosen freely within certain limits or made to suit prospective further needs, without there being any noteworthy deviation from the desired tint in the further dyeing operations. Likewise, if it is found in the course of a dyeing operation that the material already in the dyebath is not attaining the desired dyeing strength, it is easy to add fresh dyestuff while the goods are in the dyebath. Thus, there is no need to fear that the dyeing will be too strong nor is there any danger that the material will be non-uniformly dyed. The restraining action of the amine itself establishes the necessary equilibrium.

Owing to the fact that in the dyeing process of this invention the final dyeing strength is rapidly attained, the separate dyeing operations are completed in a substantially shorter period than has been possible hitherto in direct dyeing processes. Moreover, it is no longer necessary, in order to produce level dyeings, to introduce the goods into the dyebath at a low temperature and then to slowly raise the bath to the boil while moving the goods. The goods may be entered at 90° C. or a higher temperature. It is no longer necessary to move energetically either the material to be dyed or the dyeing liquor, and in spite of this level dyeings are obtained even with closely packed materials.

Dyeings on cellulose materials, which have been produced with cupriferous direct dyestuffs by the processes hitherto known in the absence of an amine of the above kind, and which are faulty, for example, are too strong or are unlevel, can in some cases be very easily rectified by the present process, even in the same dyebath and without loss of dyestuff. By the addition to the dyebath of an amine having the constitution mentioned above, the greater part of the dyestuff can be removed from the fiber. When the dyeing is too strong, the excess of dyestuff can be removed by withdrawing a corresponding quantity of the dye liquor, which may, if desired, be replaced by water. Then advantageously after the dyebath has been cooled to some extent, the action of the amine can be reduced by an addition of formaldehyde and

dyeing is repeated in the same bath with the dyestuff that is at present in solution.

The following examples illustrate the invention, the parts and percentages being by weight unless otherwise stated and the relationship of parts by weight to parts by volume being the same as that of the kilogram to the liter. The dyestuffs used in these examples are in the ordinary commercial form, which have been brought to a predetermined standard strength by the addition of a salt.

*Example 1*

A dyebath is prepared from 6000 parts of water, 15 3 parts of the copper compound of the dyestuff obtained by coupling 2 molecular proportions of diazotized 2-amino-1-hydroxybenzene-4-sulfonic acid amide with 1 molecular proportion of 5:5'-dihydroxy-2:2'-dinaphthylamine-7:7'-disulfonic acid, the copper compound containing 2 atoms of copper bound in complex union per molecule of dyestuff, 30 parts of crystalline sodium sulfate and 6 parts of 1:2-di-( $\beta$ -hydroxyethylamino)-ethane. 100 parts of wetted cotton are entered 20 into the dyebath at the boiling temperature, and boiling is continued for  $\frac{1}{4}$  hour. There are then added in several portions 6 parts by volume of formaldehyde solution of 30 per cent strength, and dyeing is continued at the boil for a further 45 minutes. In this manner there is obtained a very well through-dyed and level violet dyeing. The dyeing is of the same strength as a dyeing produced by the usual methods with 3 25 parts of the aforesaid cupriferous dyestuff.

By omitting the formaldehyde addition in the above dyeing procedure, there is obtained after about 5 minutes a dyeing of which the strength corresponds to that of a dyeing obtained by the usual methods with 0.4 part of the dyestuff (0.4 per cent. dyeing) without the addition of the amine. By boiling for a longer time the dyeing is not strengthened. After removing from the dyebath the 100 parts of cotton so dyed, it is possible to dye successively in the same bath without any further addition of dyestuff three further portions of 100 parts of cotton within a period of 15 minutes for each dyeing operation, practically the same dyeing strength (0.4 per cent) being obtained in each case. If after these 30 four dyeing operations in the same bath, it is desired to produce further dyeings of the same strength a further 1 part of the dyestuff must be added to the dyebath in order to bring the ratio of the quantity of dyestuff to amine concentration to its original value.

The dyeing strength obtained in dyeing as described above without the addition of formaldehyde is dependent on temperature to the extent that at a dyeing temperature of 20° C. a 35 dyeing is obtained of about double the strength of a dyeing obtained at the boiling temperature. From this it will be seen that a true equilibrium has been established, since a shifting of the equilibrium in favor of the dyestuff dissolved in the dyebath at a higher temperature is always possible, whereas the possibility of a longer time being required to establish the equilibrium at a high temperature than is required at a low temperature seems to be out of the question.

On the other hand the concentration of the dyestuff in the dyebath is variable within wide limits without affecting the strength of the dyeing produced. Thus, at a liquor ratio of 1:20 practically the same dyeing strength is obtained 40 as at a liquor ratio of 1:200.

The extent of the restraining action is dependent on the concentration of amine in the dye-bath. If, instead of the above concentration of 1 part of 1:2-di-( $\beta$ -hydroxyethylamino)-ethane in 1000 parts by volume of dye liquor, a concentration of 0.3 part in 1000 parts by volume is used there is obtained a 1 per cent. dyeing. With 1.6 parts of amine in 1000 parts by volume there is obtained a 0.3 per cent. dyeing. Further values, which illustrate how the dyeing strength depends on the concentration of amine for the above mentioned dyestuff (A) and three other dyestuffs (B, C and D), will be apparent from the curves given in the accompanying drawing. In the drawing

X=concentration of the 1:2-di-( $\beta$ -hydroxyethylamino)-ethane, that is to say, the number of parts in 1000 parts by volume of dye liquor,  
Y=the strengths of the dyeing produced, expressed as percentages of the dyestuff used which in normal dyeing processes yield the same dye strengths as the dyeings obtained with the amine addition, that is to say the dyeing strengths which correspond to the dyeing strengths obtained in dyeing 100 parts of cotton with Y parts of dyestuffs without the addition of amine.

A=the complex copper compound of the formula



(See the first paragraph of this example)

B=the complex copper compound of the formula



C=the complex copper compound of the formula



D=the complex copper compound of the formula



(See Example 2)

In the above formulae the method of representing the copper in complex union is one which

sumed therefrom as to the actual distribution of electro and covalencies or as to the state of hydration of the complex compounds.

For a given concentration of amine the strength of the resulting dyeing is approximately proportional to the dyestuff content of the dye-bath. Thus, if in this example, there is used, instead of 3 parts, 8 parts of dyestuff, there is obtained a 1 per cent. dyeing, with 16 parts of dyestuff there is obtained a 2 per cent. dyeing.

Similar results are obtained when in the above processes the 1:2-di-( $\beta$ -hydroxyethylamino)-ethane is replaced by one of the amines of the formulae



and



#### Example 2

100 parts of cotton are dyed with 3 parts of the complex copper compound of the disazo dyestuff from 2 molecular proportions of diazotized 2-amino-1-hydroxybenzene-4-sulfonic acid and 1 molecular proportion of 5:5'-dihydroxy-2:2'-dinaphthyl-urea-7:7'-disulfonic acid by one of the usual methods for direct dyeing and in the absence of an amine. By entering the cotton which has thus been dyed a violet tint into a



boiling bath which contains in 6000 parts of water 6 parts of 1:2-di-( $\beta$ -hydroxyethylamino)-ethane, and treating the material for about  $\frac{1}{4}$  hour at the boiling temperature, the dyestuff can be practically completely removed. By the addition of formaldehyde the dyestuff removed can be again taken up by the fiber in the same dye-bath.

#### Example 3

1 part of the nickel compound of the dyestuff of the formula



is frequently used. However, nothing can be as-

is dissolved in 100 parts of hot water.

7

10 parts of this stock solution are added to a dyebath consisting of 260 parts of water and 30 parts of sodium sulfate solution of 10 per cent strength. Then 0.3 part of 1:2-di-( $\beta$ -hydroxyethylamino)-ethane are added.

10 parts of cotton are entered into the dye-bath at the boiling temperature and a quarter of an hour later 3 parts of a formaldehyde solution of 3.3 per cent strength are gradually added in the course of a quarter of an hour. Dyeing is then continued for another 30 minutes at the same temperature. The cotton is then rinsed, centrifuged and dried. There is thus obtained a reddish blue dyeing of outstanding levelness and penetration.

8

hydroxyethylamino)-ethane and the dyestuff of the formula



10 5. A process for dyeing cellulose fibers with direct-dyeing metalliferous azo dyestuffs which comprises using a dyebath containing 1:2-di-( $\beta$ -hydroxyethylamino)-ethane and the dyestuff of  
15 the formula



What is claimed is:

1. A process for dyeing cellulose fibers with direct-dyeing metalliferous azo dyestuffs containing in complex union a metal having an atomic number ranging from 28 to 29 which process comprises using a dyebath containing an aliphatic amine of the formula



in which  $R_1$  indicates a member selected from the group consisting of a hydrogen atom, an alkyl group with at most three carbon atoms and a hydroxymethyl group,  $R_2$  indicates a member selected from the group consisting of a hydrogen

25 6. A process for dyeing cellulose fibers with direct-dyeing metalliferous azo dyestuffs which comprises using a dyebath containing 1:2-di-( $\beta$ -hydroxyethylamino)-ethane and the dyestuff of the formula



7. A process for dyeing cellulose fibers with direct-dyeing metalliferous azo dyestuffs which comprises using a dyebath containing 1:2-di-( $\beta$ -hydroxyethylamino)-ethane and the dyestuff of the formula



atom and a methyl group and  $n$  represents a whole number which is at most 4.

whole number which is at least 4.

2. A process for dyeing cellulose fibers with direct-dyeing metalliferous azo dyestuffs containing in complex union a metal having an

8. A process for dyeing cellulose fibers with direct-dyeing metalliferous azo dyestuffs which comprises using a dyebath containing 1:2-di-( $\beta$ -hydroxyethylamino)-ethane and the dyestuff of the formula



atomic number ranging from 28 to 29 which process comprises using a dyebath containing 1:2-di-(*o*-hydroxethylamino)-ethane.

3. A process for dyeing cellulose fibers with direct-dyeing cupriferous azo dyestuffs which comprises using a dyebath containing 1:2-di-( $\beta$ -hydroxethylamino)-ethane.

4. A process for dyeing cellulose fibers with direct-dyeing metalliferous azo dyestuffs which comprises using a dyebath containing 1:2-di-(8-

9. A dyebath which contains a direct-dyeing metalliferous azo dyestuff containing in complex union a metal having an atomic number ranging from 28 to 29 and also contains an aliphatic 70 amine of the formula



75 in which  $R_1$  indicates a member selected from

the group consisting of a hydrogen atom, an alkyl group with at most three carbon atoms and a

15. A dyebath which contains the metalliferous azo dyestuff of the formula



hydroxymethyl group,  $R_2$  indicates a member selected from the group consisting of a hydrogen atom and a methyl group and  $n$  represents a whole number which is at most 4.



10. A dyebath which contains a direct-dyeing metalliferous azo dyestuff containing in complex union a metal having an atomic number ranging from 28 to 29 and also contains 1:2-di-( $\beta$ -hydroxyethylamino)-ethane.

11. A dyebath which contains a direct-dyeing cupriferous azo dyestuff and also contains 1:2-di-( $\beta$ -hydroxyethylamino)-ethane.

12. A dyebath which contains the metalliferous azo dyestuff of the formula



and also contains 1:2-di-( $\beta$ -hydroxyethylamino)-ethane.

13. A dyebath which contains the metalliferous azo dyestuff of the formula



and also contains 1:2-di-( $\beta$ -hydroxyethylamino)-ethane.

14. A dyebath which contains the metalliferous azo dyestuff of the formula



and also contains 1:2-di-( $\beta$ -hydroxyethylamino)-ethane.

25 17. Process for the establishment of an equilibrium between the dyestuff in a dyebath and the dyestuff on the cellulose fibers in such bath, comprising the treatment of cellulose fibers dyed 30 with a direct-dyeing metalliferous azo dyestuff containing in complex union a metal having an atomic number from 28 to 29 in a bath containing, in addition to the dyestuff on the fiber, an aliphatic amine having at least 2 nitrogen atoms bound to 2 carbon atoms and having at least 2 hydroxyl groups.

40 JACQUES WEGMANN.  
KARL MENZI.

References Cited in the file of this patent

UNITED STATES PATENTS

| Number       | Name              | Date           |
|--------------|-------------------|----------------|
| 55 2,092,429 | Straub -----      | Sept. 7, 1937  |
| 2,155,135    | Kartaschoff ----- | Apr. 18, 1939  |
| 2,256,806    | Kern -----        | Sept. 23, 1941 |

FOREIGN PATENTS

| Number     | Country             | Date          |
|------------|---------------------|---------------|
| 60 307,948 | Great Britain ----- | Mar. 14, 1929 |